

3,519,625

**ETHERIFIED METHYLOLATED MELAMINES AND  
PROCESS FOR FINISHING CELLULOSIC TEX-  
TILE MATERIAL THEREWITH**

Michael Thomas Beachem, Somerset, and Frederic Houghton Megson, Martinsville, N.J., assignors to American Cyanamid Company, Stamford, Conn., a corporation of Maine

No Drawing. Filed Mar. 13, 1967, Ser. No. 622,400  
Int. Cl. C07d 55/22

U.S. Cl. 260—249.6

5 Claims

**ABSTRACT OF THE DISCLOSURE**

This invention relates to new and etherified methylolated melamines and their use on cellulosic textile materials dyed with direct dyes. The new etherified melamines impart crease-resistance to such materials and the light-fastness of the direct dyes is improved.

This invention relates to new compounds and to textile finishes for dyed cellulosic textile materials. More particularly, it relates to etherified melamine-formaldehyde precondensates and their use on cellulosic textile materials dyed with direct dyes. Still more particularly, it relates to the use of new etherified methylolated melamines of the Formula I:



wherein "alkyl" is a lower-alkyl group (1-4 C atoms) and R is hydrogen, alkyl of up to 18 C atoms, phenyl or phenyl(lower-alkyl), any of the phenyl or said R groups, especially when R is aryl, having up to two inert radicals, such as lower-alkyl and lower-alkoxy groups.

The use of aminoplast resins to impart crease-resistance to cellulosics is well-known. These resins perform their function economically and efficiently without adversely affecting many of the other desirable properties of cellulosics, such as, for example, fabric hand, soil resistance or fabric durability. However, aminoplast resins do in some cases have an adverse effect on color stability of dyed cellulosics. Thus, it is well-known that aminoplast crease-preventing finishes can cause accelerated fading of many direct dyes, i.e., the lightfastness of cellulosic textile material dyed with direct dyes is often reduced when the dyed material is after-treated with an aminoplast resin or reactant, such as a urea-formaldehyde or a melamine-formaldehyde condensate. Commercial resins which have been shown to cause fading of certain direct dyes include hexa(methoxymethyl)melamine, polymethyloolurea with slight degree of methylation, blends of partially methylated hexamethylolmelamine and urea-formaldehyde reaction products, and methylated trimethylolmelamine.

In view of the widespread use of both direct dyes and

aminoplast resins on cellulosics, it is extremely undesirable to have the use of the resin for its purpose, restrict the functioning of the dye for its purpose. It is therefore an object of the present invention to provide a means of treating direct-dyed cellulosics with aminoplast resins whereby crease-resistance is imparted to the cellulosic with no substantial reduction in lightfastness. It is a further object to provide cellulosics which have been direct dyed and have improved lightfastness, while also exhibiting good crease-resistance by virtue of treatment with a particular aminoplast resin textile improving agent. Other objects will be apparent from the ensuing description of this invention.

It has now been discovered in accordance with this invention that etherified methylolated melamines of Formula I impart crease-resistant properties to cellulosic textile materials without adversely affecting the lightfastness of such material dyed with direct dyes. This is a surprising discovery since cellulosics dyed with direct dyes are normally adversely affected as to lightfastness when after-treated with aminoplast textile finishes.

The textile finishing aminoplast resins used in this invention are applied to direct-dyed cellulosic textile materials by standard procedures, as by dipping, padding, spraying, etc., and the finishes are converted to an insoluble state by heating the treated fabrics in the presence of a catalyst. The dyed materials thus treated exhibit crease-resistant and wrinkle-recovery properties, and a lightfastness equal to, or even better than the untreated, dyed material.

The compounds of Formula I can be made by reacting an N-halomethylmelamine of Formula II with an alkali metal salt of Formula III as above:

wherein X is chlorine or bromine, M is an alkali metal, and "alkyl" and R are as defined above for Formula I. The compounds of Formula II and a process for their manufacture are disclosed and claimed in U.S. Pat. No. 3,317,529, issued May 2, 1967 to Beachem et al.

Representative N-halomethylmelamines of Formula II which can be used in this invention include N-chloromethyl-N,N',N',N'',N''-pentakis(methoxymethyl)-2,4,6-triamino-s-triazine, N-bromomethyl-N,N',N',N'',N''-pentakis(methoxymethyl)-2,4,6-triamino-s-triazine, N-bromomethyl-N,N',N',N'',N''-pentakis(ethoxymethyl)-2,4,6-triamino-s-triazine, N-chloromethyl-N,N',N',N'',N''-pentakis(butoxymethyl)-2,4,6-triamino-s-triazine, etc.

Representative compounds of Formula III include the sodium salts of benzyl alcohol, p-methylbenzyl alcohol, p-ethylbenzyl alcohol, etc.

The reaction of compounds of Formula II with compounds of Formula III is carried out with or without a solvent, although it is preferable to use a solvent, particularly the alcohol from which the said alkali metal salt is prepared. The reaction is conveniently carried out at room temperature, although any temperature between the freezing and boiling points of the reaction mixture may be used. Equimolar amounts of reactants can be advantageously used, although an excess of either can be present without adverse effect.

The cellulosic textile materials include fibers, threads, yarns, knitted and woven cloth as well as non-woven fabrics and felted materials. These cellulosic materials will normally contain at least 50% cellulosic fibers, such

## 3

as cotton, viscose, cuprammonium rayons, linen, hemp, jute and ramie, either alone or mixed with themselves or other fibers.

The cellulosic textile materials will be dyed with the class of azo dyes known as direct dyes and so classified in the Color Index, second edition. Such dyes are characterized as anionic dyes having affinity for cellulosic fibers when applied from an aqueous dyebath containing an electrolyte. They are mainly azo dyes containing sulfonic acid groups as the sodium salts. Representative direct dyes are Direct Yellow 6 (C.I. 4001), Direct Yellow 11 (C.I. 40000), Direct Orange 26 (C.I. 29150), Direct Red 1 (C.I. 22310), Direct Red 31 (C.I. 29100), Direct Blue 2 (C.I. 22590), and Direct Green 1 (C.I. 30280).

The dyed materials are treated with the textile finishes of this invention using aqueous or organic solvent solutions or dispersions which can be applied by spraying, dipping or padding according to well-known procedures. Between 0.5% and 40% solutions or dispersions are normally used. The amount of finish on the textile material can be varied, usually between 0.5% and 40% based on the weight of the textile material, with amounts between 2.5% and 15% preferably being used for practical crease-resistant and wrinkle-recovery properties. The treated fabrics are dried and then heated, preferably in the presence of a catalyst, to effect insolubility of the precondensate on the fabric (cross-linking, etc). Curing temperatures between 275° and 400° F. for periods of about 20 minutes to 30 seconds are normally used.

Suitable catalysts includes those normally used for melamine-formaldehyde condensates and their etherates. These include the metal salts such as magnesium chloride, zinc nitrate and zinc chloride, ammonium salts such as ammonium sulfate, ammonium chloride, and organic amine hydrochlorides. In the case of magnesium chloride, the amount is between about 4.5% and 24%, preferably between 9% and 15%, of the anhydrous salt based on the weight of the precondensate.

The treated dyed fabric obtained by this convention will be found to have good wrinkle-recovery and crease-resistance normally required for commercial cellulosics. In addition, advantageously, they will be found to possess lightfastness not previously attained with aminoplast resin-treated direct-dyed cellulosics.

The following examples are presented to further illustrate this invention.

## EXAMPLE 1



A solution of 39.8 parts (0.01 mole) of N-chloromethyl - N,N',N'',N'' - pentakis(methoxymethyl)-2,4,6-triamino-s-triazine in 54.1 parts (0.50) mole of benzyl alcohol is added slowly to the reaction mixture of 54.1 parts (0.50 mole) of benzyl alcohol and 2.39 parts (0.105 mole) of sodium at 25-30° C. After a reaction period of about 24 hours, 100 parts of water is added. The organic layer is washed with 10% aqueous sodium hydroxide, 5% sodium chloride solution and a 50:50 (by volume) mixture of methanol and water. The unreacted benzyl alcohol is removed by vacuum distillation. The product, a viscous liquid, is N-(benzyloxymethyl)-N,N',N'',N''-pentakis - (methoxymethyl)-2,4,6-triamino-s-triazine.

## 4

## EXAMPLE 2



The procedure of Example 1 is followed, substituting an equivalent amount of N-chloromethyl N,N',N'',N''-pentakis(ethoxymethyl)-2,4,6-triamino-s-triazine for the N - chloromethyl - N,N',N'',N'' - pentakis(methoxymethyl)-2,4,6-triamino-s-triazine. The product is N-(benzyloxymethyl) - N,N',N'',N'' - pentakis(ethoxymethyl)-2,4,6-triamino-s-triazine.

## EXAMPLE 3



The procedure of Example 1 is followed, substituting an equivalent amount of p-methoxybenzyl alcohol for the benzyl alcohol. The product is N-(p-methoxybenzyl)-N,N',N'',N''-pentakis(methoxymethyl)-2,4,6-triamino-s-triazine.

## EXAMPLE 4



The procedure of Example 1 is followed, substituting an equivalent amount of p-ethylbenzyl alcohol for the benzyl alcohol. The product is N-(p-ethylbenzyl)-N,N',N'',N''-2,4,6-triamino-s-triazine.

## EXAMPLE 5

Pad baths are prepared containing 6.25% of precondensate solids and 12% magnesium chloride based on the precondensate solids in the bath.

## Pad Bath A

N - (benzyloxymethyl) - N,N',N'',N'' - pentakis(ethoxymethyl)-2,4,6-triamino-s-triazine, the product of Example 1, in 85% aqueous dimethylformamide.

## Pad bath B

N,N,N',N'',N'' - hexakis(methoxymethyl) - 2,4,6-triamino-s-triazine in water, for purposes of comparison.

The pad baths are applied to 80 x 80 cotton percale at 5% O.W.F. of precondensate solids by standard padding procedure using 80% wet pickup. The treated fabrics are dried for 2 minutes at 225° F. and the finish is cured by heating the fabric at 350° F. for 1.5 minutes.

The wrinkle recovery of the treated fabrics and a sample of untreated fabric is measured on a wrinkle recovery tester following tentative test method 66-1959T, described on page B-143 of the 1964 Technical Manual and Year Book of the American Association of Textile Chemists and Colorists.

The strength loss due to retained chlorine is measured by standard test method 92-1962, described on page B-102 of the above reference, before and after five acid rinses.

The acid rinses ("acid sours") are carried out by immersing the fabric in an aqueous solution of zinc fluorosilicate followed by drying.

The measurements of finishes A and B corresponding to pad baths A and B, respectively, show the finishes to be about equivalent in degree of wrinkle recovery, but

